

Patented Dec. 22, 1931

1,837,279

# UNITED STATES PATENT OFFICE

WILLIAM J. MCGILL, OF WHITING, INDIANA, ASSIGNOR TO STANDARD OIL COMPANY, OF WHITING, INDIANA, A CORPORATION OF INDIANA

## LUBRICANT OIL

No Drawing.

Application filed November 12, 1926. Serial No. 148,100.

In accordance with the present invention the cold test, pour test or equivalent inspection test of viscous hydrocarbon oils such as those used primarily for lubricating purposes is lowered by the addition to such oils of compounds of hydroxystearic acid from the group including hydroxystearic acid, zinc hydroxystearate and magnesium hydroxystearate. The proportion of the hydroxystearic acid compound supplied is controlled in proportion to the lowering in cold or pour test desired. Ordinarily the amount required is less than 40 to 50 grams per liter of oil.

For example, with a viscous hydrocarbon lubricant oil of 180 sec. Saybolt (100° F.) viscosity having a pour test of 30 to 35° F., the addition of 5 grams of hydroxystearic acid or zinc hydroxystearate reduces the pour test to below 10° F. The addition of 10 grams hydroxystearic acid per liter of oil reduces the pour test to 2° F.; the addition of 10 grams magnesium hydroxystearate per liter of oil reduces the cold test to 5° F. and somewhat greater reductions in cold tests were secured by the addition of larger amounts of the hydroxystearic acid compounds.

I claim:

- 30 1. A lubricant oil comprising a viscous hydrocarbon oil and not more than 50 grams per liter of hydroxystearic acid.
- 35 2. The method of lowering the pour point of a viscous hydrocarbon oil which consists in supplying therein a compound of the group consisting of hydroxystearic acid and the zinc and magnesium compounds thereof.
- 40 3. A lubricant oil comprising a viscous hydrocarbon oil and not more than 50 grams per liter of a pour point depressing hydroxystearic acid compound.
- 45 4. The method of lowering the pour test of viscous hydrocarbon oils which consists in supplying thereto a pour point reducing hydroxystearic compound.

5. A lubricant oil comprising a viscous hydrocarbon oil and not more than 50 grams per liter of a pour point reducing hydroxystearic compound.

6. The method of reducing the pour test of viscous hydrocarbon oils which comprises supplying therein up to 50 grams per liter of a hydroxystearic compound of the group consisting of hydroxystearic acid and the zinc and magnesium compounds thereof.

7. The method of lowering the pour point of a viscous hydrocarbon oil which comprises supplying thereto up to 50 grams per liter of a hydroxystearic compound.

8. The method of lowering the pour point of a viscous hydrocarbon oil which comprises supplying thereto up to 50 grams per liter of hydroxystearic acid.

9. The method of lowering the pour test of a viscous hydrocarbon oil which comprises supplying therein a metallic compound of hydroxystearic acid selected from the group consisting of the zinc and magnesium soaps of hydroxystearic acid.

10. The method of reducing the pour test of viscous hydrocarbon oils which comprises supplying therein up to 50 grams per liter of a metallic compound of a hydroxystearic acid selected from the group consisting of the zinc and magnesium soaps of hydroxystearic acid.

11. A lubricant compound comprising a viscous hydrocarbon oil and a metallic compound of hydroxystearic acid selected from the group consisting of the zinc and magnesium soaps of hydroxystearic acid.

12. A lubricant oil comprising a viscous hydrocarbon oil and not more than 50 grams per liter of a compound selected from the group consisting of zinc and magnesium hydroxystearates.

13. The method of lowering the pour test of a viscous hydrocarbon oil which comprises supplying therein zinc hydroxystearate.

14. The method of lowering the pour test of a viscous hydrocarbon oil which comprises

50

55

60

65

70

75

80

85

90

supplying therein magnesium hydroxystearate.

15. A lubricant compound comprising a viscous hydrocarbon oil and zinc hydroxystearate.

16. A lubricant compound comprising a viscous hydrocarbon oil and magnesium hydroxystearate.

17. A lubricant oil comprising a hydrocarbon oil and from 5 to 50 grains per liter of a pour point reducing hydroxystearic compound.

18. A lubricating oil comprising a hydrocarbon oil and from 5 to 50 grams per liter of a pour point reducing compound selected from the group consisting of hydroxystearic acid and the zinc or magnesium compound thereof.

WILLIAM J. McGILL.

20

25

30

35

40

45

50

55

60

65